

B. E. REUTER.

SOAP AND CANDLE AND IMPROVED PROCESS OF MAKING THE SAME.

APPLICATION FILED APR. 9, 1914.

1,248,402.

Patented Nov. 27, 1917.



Witnesses:

Witnesses:  
Geo. C. Cheney  
Robert F. Bracke

Inventor  
Balthazar E. Reiter  
By  Attorney A. Williams

# UNITED STATES PATENT OFFICE.

BALTHASAR E. REUTER, OF CHICAGO, ILLINOIS.

## SOAP AND CANDLE AND IMPROVED PROCESS OF MAKING THE SAME.

1,243,403.

Specification of Letters Patent. Patented Nov. 27, 1917.

Application filed April 9, 1914. Serial No. 830,588.

To all whom it may concern:

Be it known that I, BALTHASAR E. REUTER, a citizen of the United States, residing at Chicago, in the county of Cook and State of Illinois, have invented a new and Improved Soap and Candle and Improved Process of Making the Same, of which the following is a specification.

I have discovered that a soap may be made within the principle of the process of my Patent No. 1,068,079, dated July 22, 1913, which is a new article of manufacture in that it is a normal hard soap, which, after aging, on exposure to air and light does not substantially darken or deepen in color.

Thus, the new soap of my manufacture, identified by the test below set forth, when removed from its packing box, where air and light are largely excluded, and placed upon the dealer's shelf, or put into use, does not turn substantially darker in color, as heretofore, but may even become lighter in color.

I have perfected the process of said Patent No. 1,068,079 in such manner as to insure obtaining said article of manufacture, and I will therefore proceed to repeat the description of the process of said patent in such perfected form, and then describe the test which I have worked out for identifying this new article of manufacture.

It has been known that contact with the air increased the discoloration in the fatty acids, but no successful means has ever been described, so far as I know, of applying the catalytic saponification art to the manufacture of commercially white or whitish finished product which after an appreciable length of time would not discolorize under the influence of air and light.

I have discovered that by (1) dividing the boiling into sections, and (2) removing the ribbon or the glycerin liquid (and preferably both) of the settling operation, between successive boilings, and (3) excluding air, I can obtain fatty acids, the soap from which will not be substantially discolorized under the conditions existing in commercial usage and handling.

I may employ an apparatus like that shown in the accompanying diagrammatic drawing, which may be described as follows:

A is the saponification tank in section, it may be constructed of iron with lead lining, or of wood with lead lining, or of any acid-resisting material. It converges to the

bottom outlet. B is the glycerin water tank into which the outlet 12 from the tank A discharges.

1 is the new form of agitator which is the subject of the application of Paul G. Kaiser and B. E. Reuter, filed November 20, 1913, Serial No. 802,025. Steam entering the body 1 of the agitator through the pipe 21 draws the contents of the tank in at the bottom, as indicated by arrow 22, and discharges it at the top as indicated by the arrows 23; thus circulating the contents of the tank over and over again through the agitator and serving both for heating and agitation. Other forms of agitator may be used, but I prefer this form since it produces quicker results and is more economical to operate and to construct.

2 is a steam seal pipe for admitting steam into the space at the top of the tank above the mixture to prevent air from entering the tank. 3 is a steam pipe of lead or brass provided with a perforated coil 18 for heating the mixture by admission of live steam at the bottom. 4 is an exhaust or relief pipe for escape of surplus steam to prevent excessive pressure forming in the tank, its end being sealed by dipping into the small amount of water contained in pan 10, so as to prevent air entering the pipe 4. 5 is a pressure gage. 6, 7 and 8 are sample cocks for drawing samples. 9 is a manhole for entering the tank. 11 is a tank for collecting the water overflowing from the pan 10. 12 is the outlet for removing the contents of the tank or any part thereof. It may also be used for charging tank A from the bottom. 13 is a thermometer. 15 is a suitable funnel connected with the pipe 20, which extends down to near the bottom of the tank and serves for charging the tank with either or all of the materials, water, glycerids, acid, saponifier, &c. 16 is the main steam supply pipe.

After the contents have been raised to the boiling by steam from coil 18, the valve in pipe 3 is closed and the valve 24 is opened so as to admit steam into the agitator. 14, 17 is the well known sylphon steam regulator. It regulates the supply of steam to the agitator in accordance with the temperature of the contents of the tank ascertained by the mercury pipe 17.

I may produce my new article of manufacture by the process about to be described from the following glycerids separately or

- collectively: beef tallow, mutton tallow, horse fat, hog fat, butter fat, and their respective greases; also whale oil, menhaden oil, fish oil, cocoanut oil, copra oil, peanut oil, linseed oil, cotton seed oil, palm oil, palm kernel oil, soya bean oil; also the hydrogenation or hardened products of many of these materials, particularly of corn oil, linseed oil, cotton seed oil and fish oil.
- 16 As catalytic saponifiers I may use the naphthalene variety of the class known generally as the Twitchell reagent, *e. g.* such as is described in United States Patent No. 628,503 of July 11, 1899, or Patent No. 15 601,603 of March 29, 1898, or Patent No. 1,082,662 of December 30, 1913, or Patent No. 1,058,633 of April 3, 1913, or Patent No. 1,079,437 of November 25, 1913.

With the knowledge of my invention it is probable that this process may be practised with other saponifiers now or hereafter known.

The amount of catalytic saponifier to be used in order to achieve my invention in its best form may be substantially the same, but is in general somewhat less than that which has been applied in catalytic saponification processes that do not employ my invention, such as the well known Twitchell process.

30 Practice has shown that in general from 0.6% to 1% of catalytic saponifier, calculated against the quantity of fat used, is sufficient for low grades of tallow, greases, cotton or corn oil; for good grades of tallow, 35 cocoanut oil, or palm kernel oil, about one half of the above amount is generally sufficient.

In outline my present process comprises mixing a glycerid with about 20% of its weight of water, in which has been dissolved, or to which has been added say 0.2% of the weight of the fat of catalytic saponifier. This mixture is suitably heated and agitated until approximately one third of the saponification has been accomplished. It is then allowed to settle out, which settling is hastened generally by the addition of a strong sulfuric acid in small amount. When separation is complete there will be found an upper white or whitish layer of fat and fatty acids, a lower layer consisting largely of water, and an intermediate layer or ribbon of material differing in color from either of the other two. I then withdraw the lower layer and the ribbon by suitable means, leaving only the upper white or whitish layer in the apparatus. I now add the same amount of water and catalytic saponifier as before and treat until approximately another one third of saponification has been accomplished. I repeat the settling and separating operation. I now add again 20% of water and 0.2% of catalytic saponifier as before, complete the saponification, settle and separate as before.

In some cases it will be found advisable to provide the material about to undergo saponification with free sulfuric acid to the extent of about 0.2% of the water in the total mix.

The progress of the saponification is controlled in the usual manner by determining the acid value of the product.

I will now proceed to illustrate my invention by means of the following examples, but I wish to be understood as not in anywise limiting myself to the details of proportion, operation, temperatures, or times, since these may be varied within wide ranges without in anywise departing from the spirit of my invention:

#### PRODUCING FATTY ACIDS FROM TALLOW.

##### Preliminary cleansing.

Pump 15,000 pounds of tallow into the tank A; turn on the steam from pipe 3 until boiling ensues; agitate by agitator 1; add 250 pounds of sulfuric acid of 80%  $H_2SO_4$ ; continue boiling for one hour; turn off the steam and stop the agitator; settle until the acid water separates out then draw it off.

##### First boil.

Boil the tallow by means of the live steam from coil 18; when boiling is effected turn the steam on the agitator by opening valve 24; turn off the steam from coil 18 by closing the valve in pipe 3; agitate; add 3000 pounds of water and 35 pounds of the naphthalene variety of the Twitchell catalytic saponifier; add 5 to 15 pounds of the above sulfuric acid; at this point the water tests 0.3%  $H_2SO_4$ ; boil and agitate for twelve (12) hours; turn on the steam seal pipe 2; stop the agitator and let settle; during this settling prevent entrance of air into the tank by causing steam to blow into the top of the tank from the steam seal pipe 2 throughout the time that the tank is not boiling; draw off the water and the ribbon of discolored material, if any, leaving the undecomposed fat and fatty acids in the tank.

##### Second boil.

Turn on the steam in coil 18; when boiling is effected start the agitator 1; turn off the steam seal pipe 2; add 3000 pounds of water, 35 pounds of the catalytic saponifier; make water acid to the extent of 0.2% to 0.4%  $H_2SO_4$  by gradual addition of sufficient of the above sulfuric acid; boil and agitate for twelve (12) hours; proceed as under "first boil" above beyond this point.

##### Third boil.

Proceed as under "second boil" by turning on the steam in coil 18, etc.; add the same amounts of water and catalytic saponifier as before, determine the acidity and correct if need be, and repeat the boiling, agitating

and separating as under "second boil" and "first boil." The material left in the tank is the free fatty acids; the glycerin is contained in the withdrawn water layers.

5

#### Washing.

Turn on the steam in coil 18 and when boiling is effected start the agitator 1, when the seal pipe is turned off. Add 1500 pounds 10 of water, boil for thirty minutes, then close down as fully described under "first boil" and let settle; withdraw the lower layer and any discolored material as under first, second and third boil, leaving the free fatty acids in the tank.

#### Neutralizing.

Turn on the steam in coil 18, as under "washing" above, and when boiling is effected start the agitator 1, when the seal pipe 2 is turned off, add barium carbonate mixed with about 150 pounds of water and boil for fifteen minutes, or until the liquid is neutral to methyl-orange indicator; I 25 have found 35 pounds barium carbonate usually to suffice. When neutral stop the agitator, turn off all steam and let settle for one hour; draw off all watery liquid and mix with the watery liquids from the 30 preceding first, second and third boils and washing. The material in the tank comprises the free fatty acids with some adhering moisture and these are now ready for use in making soap as given below.

35 While I have above described an equal distribution of the catalyst between the three saponification operations, and prefer that form of process, I am aware that in regulating this distribution the operator 40 should have some regard to the kind and quality of stock under treatment, but as a rule if an equal distribution is departed from I have found it best to have the proportions either progressively greater or progressively smaller, or to have the first proportion intermediate in amount between the second and third.

#### PRODUCING SOAP FROM THE ABOVE PRODUCT.

50 Weigh off 2,000 pounds of the above fatty acid product; place it in a suitable tank such as a steam jacketed soap mixing machine; add thereto 1000 pounds of a caustic soda solution containing about 290 pounds 55 of  $\text{Na}_2\text{O}$  and so much more thereof as may be necessary so that the soap resulting may contain the usual small amount of free alkali; during the mixing of the fatty acid and the caustic soda they should be very 60 well intermingled; raise the temperature by means of steam to a temperature ranging from 170 degrees to 200 degrees F.; the progress of the action is controlled in the usual way by means of the usual free alkali 65 test.

The material thus produced is ready for further suitable treatment for the production of either a colored or non-colored soap in the usual way.

In lieu of the above method of making the 70 soap from the fatty acid the ordinary boiling method may be employed.

The above examples are both based upon actual factory operation, and the results there described will be certainly obtained 75 on repeating them in the amounts and under the conditions described.

In the soap making art and in the art of making fatty acids the benefits of this invention are not realized when the amount of 80 glycerid operated on in one batch is less than 10,000 pounds. My discovery and invention are of such a nature that they are easily overlooked or not taken into account in minor operations, such as laboratory and 85 investigation work, and even on small factory scales, where the unit is less than 10,000 pounds of glycerid.

My new article of manufacture may be identified by the following test, after the 90 soap has aged for a period of ten days from the time of production.

I take a bar of soap which has been wrapped in the usual commercial way, in one or more wrappings of paper, for at 95 least ten days. I cut the bar in half, remove one half and securely rewrap the other half in the paper. I now expose the removed half to the action of air and sun-light, under such conditions that the soap 100 does not come into contact with dust or other solid material, preferably by exposing this test bar to the air and sun-light under glass in any such way that the air has access to the soap, and solid particles 105 are excluded. At the end of the test period, say ten days, the exposed half is compared with the wrapped half and will be found to be not substantially darkened in color, or may even be found to be lighter in color. 110

I have not described the introduction of any bleaching agent, and when properly conducted upon proper stock no bleaching agent is necessary for the production of good results, but I do not wish to be understood as limiting myself to the exclusion of a bleaching agent. 115

By "soap" as used in this specification I means a soap which is a normal hard soap.

I am aware that the attempt has been 120 made to maintain the lightness of color not by the treatment of the soap itself, but by the addition to the soap of whitening agents, such as zinc oxid or a peroxid, such as sodium, zinc, calcium, hydrogen, and the 125 like. But I do not wish to be understood as claiming articles in which the color is maintained substantially by the admixture of such foreign materials.

It is commercially and economically prac- 130

ticable with the above process to obtain the fatty acid product substantially free from glycerin; and commercially for soap making I prefer that it be substantially free from glycerin, but I do not wish to be understood as limiting myself to the exclusion of glycerin.

#### PRODUCING STEARIC ACID SUBSTANCES.

10. The fatty acid product above obtained contains two or more fatty acids. When made from some of the starting glycerids, such as tallow, one or more of these fatty acids is a solid fatty acid, such as stearic acid. By separating this solid fatty acid or stearic acid from the other constituents of the fatty acid product, it may be sold as such, or may be used in the manufacture of candles, toilet preparations, or other articles containing solid fatty acid or stearic acid, by the same methods heretofore employed in making such articles with ordinary stearic acid.

Such articles containing solid fatty acid or stearic acid when embodying my invention are identifiable by testing in the same manner as above described for soap.

By solid fatty acid substance I refer to either the solid fatty acid itself or an article containing the same.

What I claim and desire to secure by Letters Patent of the United States is—

1. The process of producing fatty acids

which consists in successively applying to the fats or oils under treatment fractional portions of the total quantity of the saponifier employed, excluding air from contact with the material undergoing saponification and removing the "ribbon of impurity," intermediate successive applications of the saponifier.

2. The process of producing fatty acids with an organic catalyzer which consists in successively heating the fatty mixture under treatment with fractional portions of the entire quantity of the catalyzer employed for saponifying fatty mixture, excluding air from contact with the materials undergoing treatment, settling out the watery portion of the mixture between successive heatings thereof and removing the "ribbon of impurity."

3. As a new article of manufacture, a solid fatty acid substance devoid of artificial coloring material which after aging for a period of ten days after making, on exposure to air and sun-light for a period of ten days has its color diminished in intensity.

In testimony whereof I have hereunto signed my name in the presence of two subscribing witnesses.

BALTHASAR E. REUTER.

Witnesses:

M. E. McNINCH,  
E. M. Lockwood.